

## UNITED STATES PATENT OFFICE.

HERMANN WEISS, OF HILCHENBACH, GERMANY.

## PROCESS OF MAKING GLUE AND GELATIN.

SPECIFICATION forming part of Letters Patent No. 738,709, dated September 8, 1903.

Application filed November 21, 1902. Serial No. 132,834. (No specimens.)

*To all whom it may concern:*

Be it known that I, HERMANN WEISS, a subject of the German Emperor, residing at Hilchenbach, Westphalia, Germany, have invented certain new and useful Improvements in the Manufacture of Glue and Gelatin, of which the following is a specification.

In the manufacture of glue and gelatin from skins or leather according to known processes the materials used are principally the head parts removed in the treatment of the skins in the tanneries, the grain layer removed in the preparation of chamois-dressed leather, and generally all small cuttings and waste which are in suitable condition for being made into glue; but tanned leather—whether bark-tanned, chamois-dressed, or chrome-tanned—is unsuitable for the manufacture of glue, because the substances of the skin which yield the glue have been changed by the tanning materials and cannot be made into glue. Such leather is also unsuitable for the manufacture of gelatin. The utilization of the waste of such leather is therefore almost entirely confined to the manufacture of manure.

This invention has for its object to render such leather or leather waste suitable for manufacture into glue or gelatin by a suitable treatment which may be called "detanning." This treatment, as applied to chrome-tanned leather which is now coming so largely into use, is as follows: Waste of chrome-tanned leather is placed for a considerable period—say about ten days—in an acid solution. A solution of sulfuric acid of 66° Baumé, of which a forty-per-cent. watery solution is prepared, has been found the most suitable. The waste may be stirred, if desired. The waste is then removed from the acid solution, thoroughly washed, and treated with any suitable alkali, preferably milk of lime, for the purpose of removing any remaining acid. After separation of the milk of lime and repeated washing with water any remaining traces of the lime are removed by treatment with acid, particularly hydrochloric acid, and the acid is then neutralized by

solutions of suitable alkalies—for instance, soda and the like. The leather or waste thus treated may be again washed, if desired, and is ready to be made into glue or gelatin in known manner.

This invention is of great economical advantage, because a new material is found for the manufacture of glue and gelatin and also because the cost of the process may be partly covered by the preparation of chrome-salts from the chrome oxid dissolved by the sulfuric acid.

In the case of chamois-dressed or bark-tanned leather or leather tanned with any other vegetable tanning substance, the process is modified. Instead of the first treatment with acid the waste is treated with alkali, and the subsequent treatment will of course correspond.

What I claim, and desire to secure by Letters Patent of the United States, is—

1. A process for treating leather waste for manufacture of glue and gelatin, consisting in immersing the leather in an acid solution, then washing it and treating it with an alkali, separating the alkali and again washing the leather, removing all traces of the alkali by further treatment with acid, and then neutralizing the acid with solutions of suitable alkalies, again washing the leather and treating it in the known manner.

2. A process for treating leather and leather waste for manufacture of glue and gelatin, consisting in treating the leather with an alkali, then separating the alkali and again washing the leather, removing all traces of alkali by treatment with acid, and then neutralizing the acid with solutions of suitable alkalies, again washing the leather and treating it in the known manner.

In testimony whereof I have hereunto set my hand in the presence of two witnesses.

HERMANN WEISS.

Witnesses:

BERNHARD KAISER,  
CARL SCHMITT.